

## UNITED STATES PATENT OFFICE

2,421,617

METHOD OF REMOVING COATINGS FROM  
METALLIC CONDUCTORSPhyllis Holmes, Stretford, England, assignor  
to Metropolitan-Vickers Electrical Company  
Limited, a company of Great BritainNo Drawing. Application December 3, 1943,  
Serial No. 512,843. In Great Britain February  
3, 1943

3 Claims. (Cl. 134—38)

1

This invention relates to the removal of coatings from metallic conductors and more particularly to the removal of electrically insulating enamel coverings from electric conductors.

The removal of insulating enamel from electric conductors to allow of satisfactory connection, as by soldering, to other conductors, generally presents appreciable difficulties. Two methods are available and have hitherto been practiced, the one involving the mechanical scraping of the covered wire or other conductor, and the other the dissolving of the enamel by organic solvents. In the case of relatively thick conductors, appreciable time is required to effect mechanical scraping, while in the case of fine wires such as used in instrument work, the time factor is still more serious and even the most careful handling may result in mechanical damage to the wire; these difficulties are further enhanced in the case of stranded conductors especially where individual strands are to be connected to corresponding strands of another conductor, such as commonly used in radio frequency work. Where removal of the enamel covering is effected by the use of organic solvents, the efficacy depends on the type and constitution of enamel and the degree of baking or stoving to which it has been subjected. Moreover, many of the insulating enamels which have more recently entered the market are substantially insoluble in the solvents and reagents hitherto commonly employed.

Experiments carried out by the present applicant using inorganic acids, such for instance as sulfuric acid, for the removal of enamel have been found to be not entirely satisfactory, largely due to the time factor involved and the relatively dangerous nature of the acid solvent. Likewise, the use of fused inorganic salts with relatively low melting point up to about 600° C. was also found to afford little success to the solution of the problem. As regards inorganic salts with melting point of from 600° C. upwards, though in the cases of a few of the many salts tried, some degree of success was met, yet in the main, and with one outstanding exception, they were objectionable from one aspect or another, such as by reason of the excessively high melting point of the salt, or the resulting contamination, for example oxidation, of the metal conductor, or the possibility of subsequent contamination due to the presence of residual traces of the salt or its constituents, or the absence of a sound, clean boundary between the conductor and the part of the coating to be left on the conductor.

The present invention is based on the discovery

2

and selection of the one material which provides the outstandingly satisfactory solution to the problem, and the determination of the conditions in which this material is to be used.

According to the present invention, in order to remove electrically insulating enamel coating from a copper or like conductor, the enamelled part is immersed in a bath of molten potassium iodide, and, after removal of the immersed part from the bath, the conductor is bared by a simple wiping operation. While potassium iodide is neutral in reaction, and accordingly not likely to cause chemical reaction with the metal of the conductor, it is none-the-less an electrolyte, and accordingly care should be taken in wiping to remove any residual potassium iodide from the bared conductor. It has been found that a simple rub between the fingers has been sufficient completely to remove varnish and residual salt, leaving a bright chemically clean surface of copper or like conductor.

In view of the fact that potassium iodide, although stable at temperatures in the region of its melting point, which is namely 680° C., nevertheless is liable, when heated to appreciably higher temperatures, to be decomposed with the consequent liberation of iodine, it is important, in practicing the invention, that the bath of potassium iodide should be maintained at a temperature only slightly above its melting point but yet sufficiently high to produce a liquid of conveniently water-like fluidity, namely a temperature within the range of, say, from 700° C. to 750° C.

In its usual commercial form, potassium iodide is liable to decrepitate somewhat violently when heated. Thus, in preparing the bath, it is preferred to grind the commercial potassium iodide and, after fusing the ground material at a temperature of about 700° C., to regrind the fused material before charging into the pot or other receptacle for the bath, the charge being then heated to, and maintained at, a temperature of from 700° C. to 750° C.

The time period during which the coated conductor should be left in the bath will depend generally upon the gauge of the conductor and the thickness of the coating. An excessive dipping time duration may lead to slight embrittlement, which is at present thought to be hydrogen embrittlement. As a general criterion, wires of, say, 0.03 inch diameter would require to be dipped for a period of up to one or two seconds for ensuring the complete decomposition of the enamel,

However, for the finer wires the dipping time need only be about one-fifth of a second.

A very desirable feature of this invention is that a clean line or boundary of sound enamel is left between the bared conductor and the part of the conductor which is to be left covered by enamel. Moreover, it is a desirable feature of this invention that in the case of an enamelled copper wire treated according to the invention a bright chemically clean surface of copper is left which is ready for soldering without further treatment.

In practicing the invention it is preferred to use a bath of potassium iodide prepared as described, in an electrically heated and thermostatically controlled pot or other receptacle.

While the invention is eminently successful as applied to the baring of copper wires coated with the insulating enamel containing resinous compositions of the polyvinyl acetal type and sold under the trade name "Formex," which, to all intents and purposes, is insoluble in all the solvents and reagents hitherto commercially used for the removal of enamel coating, the invention is also applicable for the baring of conductors having any of the various enamel insulating coatings in present-day use.

What I claim as new and desire to secure by Letters Patent of the United States is:

1. The method of removing an electrically insulating coating comprising a polyvinyl acetal resin from an electrical conductor which com-

prises immersing the coated conductor in a bath of molten potassium iodide maintained at a temperature between 700° C. to 750° C. and for a time sufficient to effect removal of the coating from the conductor and removing any excess potassium iodide remaining on the conductor after the immersion.

2. The method of removing an electrically insulating coating comprising a polyvinyl acetal resin from a metallic conductor which comprises subjecting the coated conductor to the action of molten potassium iodide.

3. The method of removing an electrically insulating coating comprising a polyvinyl acetal resin from a copper conductor which comprises immersing the coated part from which the coating is to be removed in molten potassium iodide, and removing any excess potassium iodide remaining on the conductor after the immersion.

PHYLLIS HOLMES.

#### REFERENCES CITED

The following references are of record in the file of this patent:

#### UNITED STATES PATENTS

| Number    | Name | Date         |
|-----------|------|--------------|
| 1,714,879 | Lang | May 28, 1929 |

#### FOREIGN PATENTS

| Number  | Country       | Date          |
|---------|---------------|---------------|
| 365,425 | Great Britain | Jan. 21, 1932 |